

## UNITED STATES PATENT OFFICE

2,197,836

## MINERAL OIL COMPOSITION

Orland M. Reiff and Elwood M. Johnson, Woodbury, N. J., assignors to Socony-Vacuum Oil Company, Incorporated, New York, N. Y., a corporation of New York

No Drawing. Application October 8, 1938,  
Serial No. 234,046

10 Claims. (Cl. 87-9)

This invention has to do in a general way with mineral oil compositions and is more particularly concerned with the production of mineral oil fractions of the viscous type, such as are used for lubricants, dielectrics, etc., which have been improved by the incorporation therein of a minor proportion of an oil-miscible metalorganic compound capable of inhibiting the deleterious effects of oxidation upon the oil.

10 It is well known that the ordinary lubricating oils, such as those used in internal combustion engines, for example, are susceptible to oxidation under normal conditions of use and, as the result of such oxidation, develop substantial quantities of carbonaceous material which accumulates as sludge or "carbon deposits" impairing the free flow of the oil. This carbonaceous material also accumulates about the piston rings, causing them to stick and filling the slots in the oil rings. Oxidation of the oil also develops substantial acidity in the oil which is corrosive to metals, particularly certain types of alloy bearing metals, and in the event the oil is used as a dielectric, the development of acidity obviously reduces its dielectric efficiency.

Numerous oxidation inhibitors have been proposed for use in mineral oils and the present invention is predicated upon the discovery of a novel class of compounds or compositions having this oxidation inhibiting action and has as its primary object the production of a mineral oil composition containing one or more of the oxidation inhibiting agents falling into this general class of compounds, to be hereinafter described.

As has been previously indicated, the materials contemplated herein as mineral oil-improving agents are metalorganic compounds. More specifically, these compounds or compositions may be classified as oil-miscible metal salts of keto acids.

The keto acids from which these metal salts are derived may be formed by the reaction of the anhydrides of aliphatic or aromatic acids with aliphatic, cycloaliphatic and aromatic compounds in the presence of a Friedel-Crafts catalyst. The alkali metal salts are formed by neutralizing the acid with a hydroxide or alcoholate of an alkali metal, and the polyvalent metal salts are obtained by double decomposition of the alkali metal salts with a salt of the desired metal.

In the event the keto acids are formed from the anhydrides of aromatic dibasic acids, the aryl nucleus of the anhydride may contain mineral oil-solubilizing substituents such as hydrogen,

halogen, alkyl, aralkyl, and alkoxy radicals or groups; and in case an aromatic hydrocarbon is used as the reactant with the anhydride, such aromatic compound may also have solubilizing substituents of the type illustrated by the examples given above.

Mineral oil-soluble salts of the type contemplated herein as oil-improving agents can be formed, for example, from keto acids obtained by hydrolyzing the products prepared (a) by the reaction of polybasic acid anhydrides with hydrocarbons from petroleum such as gasoline, kerosine, gas oil, petrolatum, and waxes; (b) by the reaction of anhydrides with cycloaliphatics such as cyclohexane, methyl cyclohexane, etc., and by the reaction of anhydrides with aromatic and mixed aromatic hydrocarbons containing halogen, hydrogen, hydroxy, alkyl, aralkyl, alkoxy, or aroxy substituents, such as toluene, chlorbenzene, amyl naphthalene, amyl phenyl ether, tetrahydronaphthalene, etc.

The keto acid salts of the type contemplated by this invention may be represented by the general formula:



in which R' represents an aliphatic group, a cycloaliphatic group, an unsubstituted aromatic group, or an aromatic group having at least one substituent selected from the group consisting of hydrogen, hydroxy, halogen, alkyl, aralkyl, alkoxy, and aroxy radicals or groups; R represents an aliphatic group, an unsubstituted aromatic group, or an aromatic group which may have one or more substituents selected from the group consisting of hydrogen, hydroxy, halogen, alkyl, aralkyl, alkoxy, and aroxy radicals or groups; and M represents the hydrogen equivalent of a metal.

In the case of salts of polybasic metals, we may, by a modified procedure to be hereinafter described, form basic metal salts of the general type discussed above. Such basic salts may be represented by the general formula:



wherein R and R' have the same significance indicated above; M<sup>V</sup> represents a polyvalent metal having a valence V of two or more; n is a whole number equal to one or (v-n') and n' is a whole number equal to one or (v-n).

The metal substituents in the carboxyl groups of the keto acid salts contemplated herein as

oxidation inhibitors for mineral oils may be broadly classified as the metals belonging to the silver, copper, tin, aluminum, iron, alkali and alkaline earth analytical groups which include: 5 silver, mercury, lead, and thallium; bismuth, copper, and cadmium; sodium, potassium, and lithium; arsenic, antimony, and tin; iron, cobalt, nickel, and manganese; and barium, calcium, strontium, and magnesium, respectively. Other 10 desirable metals include: titanium, cerium, thorium, vanadium, molybdenum, tungsten, uranium, and platinum.

Procedures which may be followed in synthesizing keto acid salts of the type contemplated herein as oxidation inhibitors for mineral oil fractions are illustrated by the following examples in which we have first described the preparation of typical keto acids, which is followed by procedures for preparing the salts from such 20 acids.

#### EXAMPLE I

##### ABOYL ALIPHATIC ACIDS BY REACTION OF AROMATIC HYDROCARBONS WITH ANHYDRIDES OF ALIPHATIC 25 DIBASIC ACIDS

One mole of succinic anhydride and one mole of amyl naphthalene are dissolved in a chlorinated solvent such as tetrachlorethane, and two mols of anhydrous aluminum chloride, or other 30 suitable Friedel-Crafts catalysts, is added to the solution with stirring at room temperature. After the aluminum chloride has been added, the mixture is heated to a temperature of about 175° F. during a three-hour period to complete the 35 reaction. The reaction mixture is then hydrolyzed and purified by washing with water containing sufficient mineral acid to remove the aluminum, after which it is water-washed until neutral.

40 At this stage the keto acid can be used in the preparation of the metal salts without removal of the solvent.

Other keto aliphatic acids can be prepared by the foregoing procedure, using anhydrides of 45 other aliphatic dibasic acids such as maleic, adipic, sebatic, pimelic, and suberic acid; also another aromatic or substituted aromatic hydrocarbon may be used as the reactant with the anhydride.

#### EXAMPLE II

##### ABOYL AROMATIC ACIDS BY REACTION OF AROMATIC AND MIXED AROMATIC HYDROCARBONS WITH ANHYDRIDES OF AROMATIC DIBASIC ACIDS

55 An illustrative reaction mixture for this synthesis is one mole of phthalic anhydride, one mole of amyl naphthalene, and two mols of aluminum chloride. The conversion to the keto acid is carried out according to the above-described synthesis of keto aliphatic acid. Orthophthalic anhydride is preferred in the synthesis of keto benzoic acids, but the meta and para acid anhydrides are also applicable to the reaction and to the formation of mineral oil-soluble salts.

60 When unreacted dibasic acid remains after the formation of the keto acid, greater difficulty is encountered in its removal than in the case of the aliphatic dibasic acids. Unreacted phthalic acid can be removed by water-washing the solution of the keto acid. As a special procedure, the solvent can be removed and the product dissolved in water in the form of the sodium salt, after which the free acid can be precipitated by neutralizing the solution with a mineral acid. By 75 repeating the solution and reprecipitation of the

keto acid, complete removal of unreacted dibasic acid is insured. It is important to effect complete removal of the unreacted acid because the reaction in which the salt is formed also converts unreacted dibasic acid to the corresponding salt which will form a cloud in mineral oil. The product of this procedure, using orthophthalic anhydride and amyl naphthalene is amyl naphthoyl-o-benzoic acid.

#### EXAMPLE III

##### KETO ACIDS FORMED BY THE REACTION OF ALIPHATIC AND CYCLOALIPHATIC HYDROCARBONS WITH THE ANHYDRIDES OF DIBASIC ACIDS

An illustrative reaction mixture for this procedure is one mole of phthalic anhydride (or succinic anhydride) one mole of Stoddard solvent and two moles of aluminum chloride. The formation of the keto acids from the aliphatic and cycloaliphatic hydrocarbons is carried out by the same procedure described under Example I above, but a higher reaction temperature (about 250° F.) is desirable to complete the reaction in the specified period of time.

When low boiling aliphatic and cycloaliphatic hydrocarbons are used, it is more suitable to use the above proportions of reactants and to prolong the time of reaction. Cyclohexane, for example, can be condensed with phthalic anhydride by heating the reactants at 175° F. during a five-hour period.

#### EXAMPLE IV

##### SALTS OF KETO ACIDS

###### A. Alkali Metal Salts

Because of the tendency of the alkali metal salts to emulsify, it is advantageous to prepare such salts in non-aqueous medium. An acid of the type obtained under Examples I, II, or III above is treated with an alkali alcoholate, preferably prepared from amyl or a lower alcohol, in an amount sufficient to neutralize the carboxyl group. The reaction mixture is held at a temperature of about 300° F. during a one-hour period during which the alcohol released in the reaction is allowed to distill off to obtain the finished product.

###### B. Other Neutral Metal Salts

A keto acid of the type obtained by the procedure of Examples I, II, or III is dissolved in a suitable solvent such as a chlorinated solvent (tetrachlorethane) or a hydrocarbon solvent (Stoddard solvent, benzol, toluene, or the like). The acid solution thus formed is neutralized with an aqueous solution of sodium hydroxide (20% NaOH) using phenolphthalein as an indicator. To the neutralized solution containing the sodium salt of the keto acid is added one mole equivalent of an inorganic salt of the desired metal. The mixture is stirred for about half an hour to complete the metathesis. The metal keto acid salt solution is then water-washed and the solvent distilled off to obtain the finished product which is a salt corresponding to general Formula I.

###### C. Basic Salts of Polyvalent Metals

Salts of this type, satisfying general Formula II, are obtained by using two mole equivalents 70 of alkali hydroxide to neutralize the keto acid in the procedure of B above and thereafter forming the salts of polyvalent metals by double decomposition with an aqueous solution of an inorganic salt of the desired metal in an amount equivalent 75

to the hydroxide used. The basic cobaltous salt of amyl naphthoyl-o-benzoic acid can be prepared with reactants in the following proportions:

|                                    | Mols |
|------------------------------------|------|
| Amyl naphthoyl-o-benzoic acid..... | 1    |
| Sodium hydroxide.....              | 2    |
| Cobaltous chloride.....            | 1    |

The acid is dissolved in benzol and neutralized with NaOH solution (20% NaOH) using phenolphthalein as an indicator and thereafter adding another mole equivalent of the hydroxide. An aqueous solution of cobaltous chloride equivalent to the sodium hydroxide is then added and the reaction mixture stirred for about thirty minutes to complete the double decomposition. The finished product is obtained by further water-washing of the benzol solution to effect complete removal of the reaction salts, followed by separation from the water and distillation of the benzol diluent.

The metal salts of keto acids of the type described above are effective oxidation inhibitors for viscous mineral oil fractions and are also capable of effecting a slight increase in the viscosity of such oil.

To demonstrate the extent to which a mineral oil blend containing a keto acid salt of the type described above has been improved over the unblended oil, we have prepared a lubricant composition by blending one-fourth per cent of the cobaltous salt of amyl naphthoyl-o-benzoic acid with a mineral lubricating oil stock of 120 seconds Saybolt viscosity at 210° F., and we have made comparative tests with the oil blend and the oil alone. These tests were carried out in a single cylinder C. F. R. engine operated for twenty-eight hours at about 1200 R. P. M. with the engine-cooling medium held at a temperature of about 390° F. The oil temperature remained in the neighborhood of 150° F. during the test.

At the end of the test the piston was examined for stuck rings and ring slots filled with carbonaceous deposit. The acidity or neutralization number (N. N.) and the weight in grams of carbonaceous deposit (C. D.) in the used oil were also determined. The comparative results obtained are listed in Table I below where oil "A" indicates the oil alone and oil "B" indicates the blend.

TABLE I

| 55         | Ring condition |   |     |     |   |                        |    |   |      |     | C. D. | N.N. |  |  |
|------------|----------------|---|-----|-----|---|------------------------|----|---|------|-----|-------|------|--|--|
|            | Degrees stuck  |   |     |     |   | Slots filled (percent) |    |   |      |     |       |      |  |  |
|            | 1              | 2 | 3   | 4   | 5 | 3                      | 4  | 5 |      |     |       |      |  |  |
| 60         | Ring No.....   | 1 | 2   | 3   | 4 | 5                      | 3  | 4 | 5    |     |       |      |  |  |
| Oil A..... | 270            | 0 | 270 | 240 | 0 | 40                     | 25 | 5 | 8.92 | 3   |       |      |  |  |
| Oil B..... | 0              | 0 | 0   | 0   | 0 | 0                      | 0  | 0 | 4.3  | 0.5 |       |      |  |  |

From the foregoing results it will be seen that metal salts of keto acids of the type contemplated herein, when blended with a viscous mineral oil fraction, retard to a substantial degree the deleterious effects of oxidation. These keto acid salts may be blended with mineral oil fractions in various proportions depending on the oil fraction and the conditions under which it is to be used. In general a satisfactory product may be obtained with about one-fourth per cent of the improving agent, but amounts ranging from

one-sixteenth per cent to two per cent may be used.

We claim:

1. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid.

2. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the anhydride of a polycarboxylic acid and a hydrocarbon material.

3. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the anhydride of a polycarboxylic acid and a hydrocarbon material selected from the group consisting of aliphatic hydrocarbons, cycloaliphatic hydrocarbons, unsubstituted aromatic hydrocarbons, and aromatic hydrocarbons having substituents selected from the group consisting of hydrogen, hydroxy, halogen, alkyl, aralkyl, and aroxy groups.

4. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the anhydride of an acid selected from the group consisting of aliphatic and aromatic polybasic acids and a compound selected from the group consisting of aliphatic hydrocarbons, cycloaliphatic hydrocarbons, unsubstituted aromatic hydrocarbons and aromatic hydrocarbons having substituents selected from the group consisting of hydrogen, hydroxy, halogen, alkyl, aralkyl, alkoxy, and aroxy groups.

5. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the anhydride of a dibasic aromatic acid and an aromatic hydrocarbon.

6. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the anhydride of a dibasic aliphatic acid and an aliphatic hydrocarbon.

7. A mineral oil composition of the type adapted for use as a lubricant or the like comprising a viscous mineral oil fraction and in admixture therewith a minor proportion, sufficient to inhibit oxidation of said oil, of an oil-miscible metal salt of a keto acid formed by hydrolyzing the Friedel-Crafts condensation product of the an-

hydride of a dibasic aromatic acid and a cycloaliphatic hydrocarbon.

5 8. A lubricating oil composition comprising a viscous mineral oil fraction and in admixture therewith a minor proportion, sufficient to inhibit oxidation of said oil, of the cobaltous salt of amyl naphthoyl-o-benzoic acid.

9. A mineral oil composition of the type adapted for use as a lubricant or the like comprising a viscous mineral oil fraction and in admixture therewith a minor proportion of a metal salt of a keto acid having the general formula:



15 15 in which  $\text{R}'$  represents an aliphatic, cycloaliphatic, or aromatic hydrocarbon group or an aromatic hydrocarbon group having at least one substituent selected from the group consisting of hydrogen, halogen, hydroxy, alkyl, aralkyl, alkoxy, and aroxy groups;  $\text{R}$  represents an aliphatic hydrocarbon group, an aromatic hydrocarbon group, or an aromatic hydrocarbon group having at least one substituent selected from the group consisting of hydrogen, hydroxy, halogen, alkyl, aralkyl, alkoxy and aroxy groups; and  $\text{M}'$  represents the hydrogen equivalent of a metal.

10 10 A mineral oil composition of the type adapted for use as lubricants, dielectrics, and the like comprising a viscous mineral oil fraction and in admixture therewith a minor proportion of a metal salt of a keto acid having the 5 general formula:



10 in which  $\text{R}'$  represents an aliphatic, cycloaliphatic or aromatic hydrocarbon group of an aromatic hydrocarbon group having at least one substituent selected from the group consisting of hydrogen, hydroxy, halogen, alkyl, aralkyl, alkoxy, and aroxy groups;  $\text{R}$  represents an 15 aliphatic hydrocarbon group, an aromatic hydrocarbon group, or an aromatic hydrocarbon group having at least one substituent selected from the group consisting of hydrogen, hydroxy, halogen, alkyl, aralkyl, alkoxy, and aroxy groups;  $\text{M}'$  represents a polyvalent metal having a valence  $v$  of two or more;  $n$  and  $n'$  are 20 whole numbers less than  $v$ ,  $n$  being equal to  $(v-n')$  and  $n'$  being equal to  $(v-n)$ .

25 ORLAND M. REIFF.  
ELWOOD M. JOHNSON.

25

### Certificate of Correction

Patent No. 2,197,836.

April 23, 1940.

ORLAND M. REIFF, ET AL.

It is hereby certified that errors appear in the printed specification of the above numbered patent requiring correction as follows: Page 4, second column, line 7, claim 10, strike out the formula and insert instead the following—



line 11, same claim, for "of" read *or*; and that the said Letters Patent should be read with these corrections therein that the same may conform to the record of the case in the Patent Office.

Signed and sealed this 19th day of November, A. D. 1940.

[SEAL]

HENRY VAN ARSDALE,  
*Acting Commissioner of Patents.*

**Certificate of Correction**

Patent No. 2,197,836.

April 23, 1940.

**ORLAND M. REIFF, ET AL.**

It is hereby certified that errors appear in the printed specification of the above numbered patent requiring correction as follows: Page 4, second column, line 7, claim 10, strike out the formula and insert instead the following—



line 11, same claim, for "of" read *or*; and that the said Letters Patent should be read with these corrections therein that the same may conform to the record of the case in the Patent Office.

Signed and sealed this 19th day of November, A. D. 1940.

[SEAL]

**HENRY VAN ARSDALE,**  
*Acting Commissioner of Patents.*